

1

2,945,811

OXIDATION AND SILVER CORROSION  
RESISTANT LUBRICANTS

Andrew D. Abbott, Ross, and James H. Walker, Richmond, Calif., assignors to California Research Corporation, San Francisco, Calif., a corporation of Delaware

No Drawing. Filed Dec. 31, 1956, Ser. No. 631,474

4 Claims. (Cl. 252—32.7)

This invention pertains to lubricating oil compositions which are particularly beneficial to use where silver wearing surfaces are concerned. In particular, lubricating oil compositions of this invention are resistant to oxidation and are noncorrosive to silver wearing surfaces, as well as being noncorrosive to the conventional metal alloy surfaces.

Generally, oils of lubricating viscosity are now subjected to higher temperatures and greater conditions of wear than those which existed only a relatively few years ago. Such changes in lubricating requirements are due primarily to the many advances which have occurred in the design of automotive equipment. For example, diesel engines used in railway service are now equipped with bearings lined with pure silver metal. Also, many automobiles have valve lifters which are subject to such high loads that the bearing surfaces operate under conditions approaching boundary lubrication. Thus, new requirements have been imposed on lubricating oils so that oils which were satisfactory just a few years ago are now inadequate for proper lubrication.

Metal salts of thiophosphoric acids, particularly alkaline earth metal and zinc salts of alkyl or alkyaryl thiophosphoric acids, have long been used as additives for lubricating oils. These salts have been extremely effective in inhibiting oxidation of oils and corrosion of alloy bearings, and in imparting extreme-pressure properties to oils.

Because the above-noted salts of thiophosphoric acids cause severe corrosion of silver in engines employing silver wearing surfaces, a bi-metal dithiophosphate was developed as a lubricating oil additive to inhibit oxidation corrosion and at the same time be substantially noncorrosive to silver wearing surfaces.

Although these bi-metal dithiophosphates are extremely effective as lubricating oil additives to impart oxidation corrosion and silver metal corrosion resistance thereto, these salts have an unfavorable characteristic. After lubricating oil compositions containing these bi-metal dithiophosphates have been left standing for a period of time, a scum forms on the surface of the oil. This scum (i.e., this film of plastic-like substance) becomes so thick and firm as to be deleterious to lubricating systems in that the lines become plugged, hampering proper lubrication.

Therefore, it is a primary object of this invention to prepare lubricating oil compositions containing carbonated bi-metal salts of thiophosphoric acids, on the surfaces of which compositions no tough film will form.

In accordance with this invention, it has been discovered that the scum-forming characteristics of lubricating oil compositions containing bi-metal salts of esters of thiophosphoric acids can be inhibited by treating such lubricating oil compositions with carbon dioxide. Thus, the oxidation and silver corrosion resistant oil compositions of this invention comprise oils of lubricating viscosity having incorporated therein carbonated bi-metal salts of esters of thiophosphoric acids.

2

It is well known that oxidation corrosion attacks wearing surfaces consisting of silver-cadmium alloys. However, the silver is present in the silver-cadmium alloy in very minor percentage amount (i.e., less than 1%). The silver wearing surfaces with which we are concerned herein include wearing surfaces which contain large amounts of silver, such as silver alloys containing more than 50% silver, and including wearing surfaces of substantially pure silver.

10 By the use of the carbonated bi-metal dithiophosphates of this invention, non-scumming, oxidation-resistant lubricants noncorrosive to silver have been obtained.

As used herein, the term "bi-metal salts of thiophosphoric acids" means the product which is obtained by reacting an alkaline earth metal oxide or hydroxide with a metal salt of an ester of thiophosphoric acid, said metals being dissimilar. The term "carbonated bi-metal salts of thiophosphoric acids" means the product obtained by contacting the bi-metal salts of thiophosphoric acids with carbon dioxide.

Bi-metal dithiophosphates are obtained by reacting alkaline earth metal oxides and/or hydroxides with metal salts of esters of thiophosphoric acids of the formula



25 wherein R and R' may be alkyl radicals containing at least 8 carbon atoms, and alkaryl or aralkyl radicals containing a total of from 12 to 70 carbon atoms; and R and R' may or may not be identical. "M" is a metal of Group II of Mendeleeff's Periodic Table, preferably calcium, barium, or zinc. The metal M is not the same metal as the alkaline earth metal of the oxide or hydroxide reactants used in the formation of the bi-metal dithiophosphates. At least one of the metals of the bi-metal dithiophosphates is an alkaline earth metal.

30 The R radicals and the R' radicals can be derived from straight chain or branched chain alcohols containing at least 8 carbon atoms, or alkylphenols, wherein the alkyl radicals contain at least 6 carbon atoms; for example, n-octanol, 2-ethylhexanol, 2-propylpentanol, decanol, undecanol, dodecanol, hexadecanol, octadecanol, 35 hexylphenol, decylphenol, dodecylphenol, hexadecylphenol, octadecylphenol, dicetylphenol, 2-phenylhexanol, etc.

35 Examples of esters of thiophosphoric acids which are reacted with the alkaline earth metal oxides or hydroxides are diethyl thiophosphoric acids; didecyl thiophosphoric acid; didodecyl thiophosphoric acid; dihexadecyl thiophosphoric acid; di(decylphenyl) thiophosphoric acid; di(amylphenyl) thiophosphoric acid; di(dodecylphenyl) thiophosphoric acid; etc.

40 Improved oil solubility of the resulting bi-metal dithiophosphate is obtained when the alkaline earth metal oxide (or hydroxide), the metal salt of thiophosphoric acid is a zinc salt of esters of thiophosphoric acid, and wherein each of the ester radicals (i.e., the R and R' of the formula hereinabove) are derived from alcohols or alkylphenols containing not less than 12 carbon atoms, and not more than 25 carbon atoms (i.e., it is preferred that the total number of carbon atoms in the ester radicals is from 24 to 50).

45 For purposes of simplification, the metal of the alkaline earth metal oxide and hydroxide reactants will be termed "secondary metal," and the metal of the dithiophosphate reactant will be termed "primary dithiophosphate metal."

50 These bi-metal salts of esters of thiophosphoric acids

have molecular weights of such magnitude as to indicate the formation of complex polymeric type compounds. Molecular weight data for these compounds, as determined by sedimentation rates in an ultracentrifuge, show that the molecular weights are in the range of 150,000 to 550,000.

Suitable base oils for the compositions of this invention include a wide variety of lubricating oils such as naphthenic base, paraffin base, and mixed base mineral oils; synthetic oils, e.g., alkylene polymers, such as polymers of propylene, butylene, etc., and mixtures thereof; alkylene oxide type polymers; dicarboxylic acid esters; liquid esters of phosphorus, liquid esters of silicon (including polysiloxanes); and alkyl aromatic hydrocarbons.

The above base oils may be used individually as such or in various combinations (wherever miscible or whenever made so by the use of mutual solvents).

The carbonated bi-metal salts of esters of dithiophosphoric acids are used in lubricating oils in amounts sufficient to inhibit oxidation thereof; that is, amounts of 0.25% to 20%, by weight, preferably from 1.5% to 10%, by weight. Stated in other terms, the amounts of these carbonated bi-metal dithiophosphates may be expressed as millimols per kilogram of finished oil, based on the phosphorus content. That is, the amount of bi-metal dithiophosphate is expressed as millimols of phosphorus per kilogram of oil (i.e., "mM./kg."). Expressed in such terms, the amount of bi-metal salts of esters of dithiophosphoric acids used in lubricating oils can be from 1 millimol to 50 millimols of phosphorus per kilogram of finished oil, preferably from 4 millimols to 25 millimols.

In the preparation of the bi-metal salts of esters of dithiophosphoric acids, the monometal salts of esters of dithiophosphoric acids of the prior art can be prepared by methods known heretofore. For example, a mixture of the desired alcohol or alkylphenol and phosphorus pentasulfide is reacted with or without a solvent (e.g., petroleum naphtha) at 100° F. to 200° F. until the dithiophosphoric acid is formed. The crude acid mixture is then filtered to remove unreacted phosphorus pentasulfide, after which the resulting acid is neutralized with a metal oxide (e.g., zinc oxide) to form the metal dithiophosphate. Such simple metal salts of esters of dithiophosphoric acids can also be prepared by reacting the dithiophosphoric acid with sodium hydroxide to form the sodium salt, then precipitating the desired metal salt from a solution of the sodium salt by the addition of a metal chloride (e.g., zinc chloride or calcium chloride).

The bi-metal salts of esters of dithiophosphoric acids (e.g., barium-zinc diester dithiophosphates) are prepared by reacting a metal diester dithiophosphate with an alkaline earth metal oxide (or hydroxide) in a solvent (e.g., a lubricating oil), followed by heating to a temperature ranging from 200° F. to 450° F. (preferably from 250° F. to 375° F.), and filtering the resulting admixture.

The carbonated bi-metal dithiophosphates of this invention are obtained by contacting the above-described bi-metal salts of dithiophosphoric acids with carbon dioxide. The carbonation can be accomplished by bubbling carbon dioxide through a solution of a bi-metal dithiophosphate (e.g., a lubricating oil solution of a bi-metal dithiophosphate) at temperatures ranging from about 60° F. to about 300° F. It is preferable to prepare a concentrate of the bi-metal dithiophosphate in oil; for example, from about 15% to about 70%, by weight, of the bi-metal dithiophosphate in a lubricating oil, and bubble the carbon dioxide through the concentrate; or treat the concentrate with carbon dioxide as described hereinbelow.

The following examples illustrate the preparation of lubricating oil compositions containing such carbonated bi-metal dithiophosphates.

#### EXAMPLE 1.—PREPARATION OF BI-METAL DITHIOPHOSPHATE

A mixture of 5 pounds (0.032 pound mol) of barium oxide (92% purity) and 125 pounds (0.0625 pound mol) of a zinc di(alkylphenyl) dithiophosphate (containing 3.27% zinc, 3.0% phosphorus, and 5.78% sulfur, and wherein the alkyl radical is derived from propylene polymers having an average of 12 carbon atoms) was incorporated in a California solvent-refined paraffin base oil having a viscosity of about 140 SSU at 100° F. The whole mixture was heated in a kettle with agitation at 300–310° F. for a period of 1.4 hours. 79 pounds (0.245 pound mol) of barium hydroxide octahydrate (98% purity) was then charged at the rate of 20 pounds per hour while the temperature was maintained at 300° F. to 310° F. The barium-to-zinc mol ratio of this charge was 4.43 to 1.0. The pH of the charge (determined in a solvent consisting of 40%, by volume, of ethyl alcohol; 40% ethyl ether; and 20% water) increased from 4 to 13+. The whole mixture was agitated at 300° F. for another hour, with nitrogen flowing through the bottom of the bottle to remove residual moisture. This was followed by a final drying period of 30 minutes at 300° F. under a vacuum of 25 inches of mercury. To this mixture was added 5 pounds of Celite filter aid, after which the mixture was cooled to 250° F. and filtered.

The resulting product analyzed 1.76% zinc, 16.73% barium, 1.63% phosphorus, and 3.26% sulfur. The mol ratios based on zinc, as one, were as follows: barium, 4.52; phosphorus, 1.95; and sulfur, 3.78. The viscosity was 3838 SSU at 100° F., and 155 SSU at 210° F.

The barium-zinc di(alkylphenyl) dithiophosphate product thus formed was isolated from the lubricating oil concentrate as follows: 100 grams of the above lubricating oil concentrate was dissolved in 100 ml. of benzene. 300 ml. of C.P. acetone was added to precipitate out the compound. The solid fraction precipitating out was separated and redissolved in 100 ml. of benzene and reprecipitated with 300 ml. of C.P. acetone.

Table I hereinbelow sets forth the analysis of the reprecipitated solid, again using zinc content as the base for determining the mol ratio.

Table I

|                 | Percent By Weight | Mol Ratio |
|-----------------|-------------------|-----------|
| Zinc.....       | 3.85              | 1.0       |
| Barium.....     | 33.7              | 4.17      |
| Phosphorus..... | 3.04              | 1.67      |
| Sulfur.....     | 6.67              | 3.53      |

The bi-metal dithiophosphates can be carbonated at atmospheric pressures and ambient temperatures (e.g., room temperature; i.e., about 68° F.), or at pressures as high as, or higher than, 100 p.s.i. and temperatures as high as, or higher than, 300° F. At the higher temperatures, it is beneficial to use lower pressures; that is, pressures ranging from about atmospheric pressure to about 50 to about 75 p.s.i. For example, when the temperature is approximately 300° F. or higher, it is preferable to use pressures from about atmospheric pressure to 50 p.s.i. When it is desirable to use lower temperatures, that is, temperatures from about 60° F. to about 225° F., higher pressures may be used (for example, pressures as high as 100 p.s.i., or higher).

For purposes of this invention, it is preferred that the carbonation of bi-metal dithiophosphates be accomplished at temperatures ranging from about 60° F. to about 225° F., and pressures from about atmospheric to about 50 p.s.i.

The following examples illustrate the preparation of carbonated bi-metal dithiophosphates.

**EXAMPLE 2.—PREPARATION OF CARBONATED BI-METAL DITHIOPHOSPHATES AT ATMOSPHERIC PRESSURE**

300 grams of an oil solution (a California solvent-refined paraffin base oil having a viscosity of about 140 SSU at 100° F.) containing 60±2%, by weight, of the bi-metal dithiophosphate of Example 1, hereinabove, was carbonated by adding Dry Ice thereto at a temperature of 300° F. The whole mixture was vigorously agitated for about 2 hours. There was a constant excess of carbon dioxide in contact with the oil liquid at all times.

**EXAMPLE 3.—PREPARATION OF CARBONATED BI-METAL DITHIOPHOSPHATE AT 100 P.S.I.**

1500 grams of an oil solution (a California solvent-refined paraffin base oil having a viscosity of about 140 SSU at 100° F.) containing 60±2%, by weight, of the bi-metal dithiophosphate of Example 1, hereinabove, were charged to a closed vessel of 2500 ml. capacity. The vessel was connected to a source of carbon dioxide, and the carbon dioxide was pressured into the closed vessel, so that a constant pressure of 100 p.s.i.g. was maintained. The reactants were constantly agitated at 325±10° F. for a period of 2 hours. The reaction product was analyzed as follows:

*Table II*

|                 | Percent By Weight | Mol Ratio |
|-----------------|-------------------|-----------|
| Zinc.....       | 1.74              | 1.0       |
| Barium.....     | 13.61             | 3.7       |
| Phosphorus..... | 1.60              | 1.93      |
| Sulfur.....     | 2.47              | 2.88      |

**EXAMPLE 4.—PREPARATION OF CARBONATED BI-METAL DITHIOPHOSPHATES AT 50 P.S.I.**

1000 grams of an oil solution (a California solvent-refined paraffin base oil having a viscosity of about 140 SSU at 100° F.) containing 60±2%, by weight, of the bi-metal dithiophosphate of Example 1, hereinabove, were charged to a closed vessel having a capacity of 2500 ml. The vessel was connected with a source of carbon dioxide and the pressure within the vessel was raised to 50 p.s.i.g. by a charge of the carbon monoxide. The contents of the vessel were vigorously agitated at 225° F. for a period of 2 hours. A constant pressure of 50 p.s.i.g. was maintained by the carbon dioxide. The reaction product analyzed as follows:

*Table III*

|                 | Percent By Weight | Mol Ratio |
|-----------------|-------------------|-----------|
| Zinc.....       | 1.61              | 1.0       |
| Barium.....     | 14.60             | 4.26      |
| Phosphorus..... | 1.54              | 2.0       |
| Sulfur.....     | 3.22              | 3.88      |

37 grams of an oil solution (60%, by weight) of the bi-metal dithiophosphate of Example 1, hereinabove, was allowed to stand in a 250-ml. beaker at room temperature for four days, during which time the surface of the oil became coated with a heavy plastic-like film.

37 grams of an oil solution (60%, by weight) of the carbonated bi-metal dithiophosphate of Example 3 was placed in a 250-ml. beaker and allowed to stand for 4 days at room temperature. The surface of this oil remained clear and free from any scum or plastic-like film formation.

The carbonated bi-metal dithiophosphates are particularly effective as lubricating oil additives when the mol ratio of the secondary metal to the primary dithiophosphate metal is from about 3.7 to 1 to about 4.6 to 1 (i.e., has a value from 3.7 to 4.6).

Table IV hereinbelow presents data showing the effec-

tiveness of carbonated bi-metal salts of diesters of dithiophosphoric acids (i.e., bi-metal dithiophosphates) as oxidation inhibitors and as silver corrosion inhibitors in lubricating oil compositions.

5 The base oil, the test conditions, etc., which were used are described as follows:

The base oil in each instance was a 60 V.I. SAE 40 California base oil containing 4 millimols of a calcium petroleum sulfonate wherein the petroleum radical was obtained from a California paraffin base oil having a viscosity of 480 SSU at 100° F. To this base oil was then incorporated the additive of the table in the amounts specified therein:

15 The bi-metal dithiophosphates were prepared according to the process described in Example 1, hereinabove, by reacting barium oxide and barium hydroxide with a zinc di(alkylphenyl) dithiophosphate, wherein the alkyl radical was obtained from polypropylenes containing an average of 12 carbon atoms. The carbonated bi-metal 20 dithiophosphates were prepared according to the process described in Example 2 hereinabove.

The "silver strip test" which was used is described as follows:

A silver metal strip having the dimensions of 2½ inches 25 by ¾ inch by ⅜ inch was first cleaned with a wire brush until the strip was highly polished. The strip was weighed and the weight recorded. This highly polished silver strip was then placed in a 600 ml. beaker in such a manner that the strip was completely immersed when 30 300 grams of the oil being tested was poured into the beaker. The oil was stirred at a temperature of 300° F. for 20 hours, at which time the silver strip was removed and cleaned, first with chloroform, then with petroleum ether. The appearance of the strip was noted. Those strips which had been severely attacked were quite black.

The tested silver strip was washed in 15% aqueous solution of potassium cyanide for about 5 minutes to remove the sulfide film adhering to the strip. After the strip had been washed with potassium cyanide and dried, it 40 was weighed. The difference in weight of the original strip and the strip after the potassium cyanide wash was noted and recorded as the weight loss due to corrosion.

45 The copper-lead strip corrosion tests were run as follows: A polished copper-lead strip (obtained from a commercial bearing) was weighed and immersed in 300 ml. of test oil contained in a 400 ml. beaker. The test oil was maintained at 295° F. under pressure of one atmosphere of air and vigorously stirred with a mechanical stirrer. After 2 hours, a catalyst was added to provide the following catalytic metals (all percentages being by weight):

|                |        |
|----------------|--------|
| Iron.....      | 0.0056 |
| Lead.....      | 0.11   |
| 55 Copper..... | 0.0095 |
| Manganese..... | 0.0005 |
| Tin.....       | 0.0049 |

50 The test was continued for 20 hours, after which the copper-lead strip was removed, rubbed vigorously with a soft cloth, and weighed to determine the weight loss.

*Table IV*

| 65 | Oil No. | Additive (m.M./kg.) (Based on Metal)  |                                     | Silver Strip Corrosion, Mgs. Loss | L-4 Engine Test, Weight Loss Mg. per Whole Bearing |
|----|---------|---------------------------------------|-------------------------------------|-----------------------------------|----------------------------------------------------|
|    |         | Uncarbonated Bi-metal Dithiophosphate | Carbonated Bi-metal Dithiophosphate |                                   |                                                    |
| 70 | 1.....  | 7                                     | 7                                   | 52.6                              | 91.4                                               |
|    | 2.....  |                                       | 7                                   | 7.6                               | 38.5                                               |
|    | 3.....  | 10                                    | 10                                  | 14.3                              | 64.5                                               |
|    | 4.....  |                                       | 10                                  | 4.6                               | 8.4                                                |
|    | 5.....  | 12                                    | 12                                  |                                   | 22.5                                               |
|    | 6.....  |                                       | 12                                  |                                   | 12.0                                               |

Although the compositions of the present invention have been described above as being primarily useful as internal combustion engine lubricants, the additives herein are suitable for use in gear lubricants, ice machine oils, instrument oils, constituent oils for grease manufacture, turbine oils, and the like.

In addition to the additives noted hereinabove, the lubricating oils of this invention may contain other oxidation inhibitors, grease thickening agents, color correctors, extreme pressure agents, oiliness agents, gel modifiers, etc.

We claim:

1. A lubricating oil composition consisting essentially of a major proportion of an oil of lubricating viscosity and a carbonated bi-metal salt of a dithiophosphoric acid in an amount of about 0.25% to 20%, by weight, wherein said bi-metal salt is prepared by reacting a metal material selected from the group consisting of barium oxide and barium hydroxide with a zinc dithiophosphate of the formula:



wherein R and R' are hydrocarbon radicals selected from the group consisting of alkyl and alkaryl radicals, each radical containing from 12 to 25 carbon atoms, wherein said reaction is at a temperature of 200° F. to 450° F., followed by filtration, and carbonating at temperatures from 60° F. to 300° F., wherein said carbonated bi-metal salts of diester of dithiophosphoric acid have a molecular weight ranging from 150,000 to 500,000, and

wherein the mol ratio of barium to zinc ranges from 3.7:1 to 4.6:1.

2. The lubricating oil composition of claim 1, wherein the zinc dithiophosphate radicals are alkaryl radicals, each containing from 12 to 25 carbon atoms.

3. The lubricating oil composition of claim 1, wherein said zinc dithiophosphate is a zinc alkaryl dithiophosphate wherein each alkyl radical is derived from propylene polymers having an average of about 12 carbon atoms.

4. A lubricating oil composition consisting essentially of a major proportion of an oil of lubricating viscosity and a carbonated bi-metal salt of a diester of a dithiophosphoric acid in an amount of 0.25% to 20%, by weight, wherein said bi-metal salt is prepared by reacting a metal material selected from the group consisting of barium oxide and barium hydroxide with a zinc di(alkylphenyl) dithiophosphate, wherein said alkyl radicals are obtained from propylene polymers having an average of about 12 carbon atoms, wherein said reaction is at a temperature of 200° F. to 450° F., followed by filtration, and carbonating at temperatures from 60° F. to 300° F., wherein said carbonated bi-metal salts of diester dithiophosphoric acid have molecular weights ranging from 150,000 to 500,000, and wherein the mol ratio of barium to zinc is from about 3.7:1 to about 4.6:1.

#### References Cited in the file of this patent

#### UNITED STATES PATENTS

2,616,924 Asseff et al. ----- Nov. 4, 1952  
2,767,164 Asseff et al. ----- Oct. 16, 1956

#### FOREIGN PATENTS

723,133 Great Britain ----- Feb. 2, 1955  
1,110,712 France ----- Oct. 19, 1955